

(No Model.)

W. F. BATHO.

BASIC LINING FOR OPEN HEARTH STEEL AND IRON FURNACES.

No. 339,360.

Patented Apr. 6, 1886.

Fig. 2



Fig. 3



Fig. 1



Fig. 4



Fig. 5



Fig. 6



Fig. 7



Fig. 8.



Witnesses

W. F. Batho

Edmund S. Breen

Inventor

W. F. Batho

# UNITED STATES PATENT OFFICE.

WILLIAM F. BATHO, OF WESTMINSTER, COUNTY OF MIDDLESEX, ENGLAND.

## BASIC LINING FOR OPEN-HEARTH STEEL AND IRON FURNACES.

SPECIFICATION forming part of Letters Patent No. 339,360, dated April 6, 1886.

Application filed October 12, 1885. Serial No. 179,604. (No model.) Patented in England February 26, 1884, No. 3,921; in France May 31, 1884, No. 162,496; in Belgium June 3, 1884, No. 65,370; in Germany June 5, 1884, No. 29,488; and in Austria-Hungary May 26, 1885, No. 2,126.

To all whom it may concern:

Be it known that I, WILLIAM FOTHERGILL BATHO, a subject of the Queen of Great Britain, residing at Westminster, in the county of Middlesex, England, have invented a new and useful Improvement in Basic Linings for Open-Heart Steel and Iron Furnaces; (for which I have obtained Patents in Great Britain, No. 3,921, February 26, 1884; in France, No. 162,496, May 31, 1884; in Belgium, No. 65,370, June 3, 1884; in Germany, No. 29,488, June 5, 1884; and in Austria-Hungary, No. 2,126, May 26, 1885, and no where else,) of which the following is a specification.

15 Basic linings for open-hearth steel and iron furnaces, as prepared and applied heretofore, have had material disadvantages, and by crumbling, fluxing, and shelling such linings have lasted much less time than is desirable, 20 or should be the case for economical working. It has been proposed to add to the basic material oxide of iron, alumina, silica, and other agents with the object of strengthening the lining. When, however, sufficient of the said 25 agents is used to cause the lining to flux to any depth, it is apt to and does flux too much and melts down, whereas a smaller quantity of the said agents in admixture causes the surface to crumble or fall away in shells.

30 Now the object of my invention is to provide basic linings for open-hearth steel and iron furnaces which shall last longer than any hitherto used, and hence will, in the same furnace insure the production of steel and iron at a material reduction in cost.

35 The invention consists, essentially, in making basic linings for open-hearth and other steel and iron furnaces of an oxide of calcium, magnesium, barium, or strontium, or an admixture of these combined with comparatively finely-divided metallic steel or iron in such manner that the particles of steel or iron come up to and form part of the wearing-surface in quantity sufficient to form the necessary flux, 40 and yet serve as a bond to the basic material.

45 In carrying my invention into practice, lime or other base or basic admixture is burned and shrunk in any known suitable way, is afterward reduced to a more or less finely-divided condi-

tion, and is applied in the furnace with steel or iron wire cuttings, by preference twisted or bent, well mixed among the mass. The steel or iron wire cuttings come to the surface so as to produce during working a glaze or skin which by oxidation enhances the life of the lining. 50 The wire acts also as a mechanical means of holding the lining material together. About ten per cent. of fine steel or iron wire cut into lengths of from one-half an inch to one and one half inch mixed with the base is found to 55 answer well, more particularly so when uniformly mixed or arranged.

I am aware it has been proposed to bind basic linings to furnace-frames by metal locking-pieces; but such arrangement falls far 60 short of the double advantage of protecting the surface and providing a mechanical bond throughout; also, that it has been proposed to mold iron borings into bricks with lime and water, or other binding material, for convenience in transportation and remelting; also, 65 that it has been proposed to make crucible cast-steel of a batch consisting of granulated cast-iron, iron ore, and small pieces of wrought-iron; also, that it has been proposed to make 70 a fettling or fix for puddling-furnaces composed of equal parts of mill-cinder, hammer-slag, and cast-iron, burned together in any suitable manner. I claim none of these things, 75 because they are not lime-linings, and do not have the functions of and are incapable of use as lime-linings; nor is the metallic iron in the above instances combined with the other ingredients for the same purpose as I combine it with the basic materials with which I use it. By 80 the use of the term "lime" in the claims I mean to include not only oxide of calcium, but also magnesium, barium, and strontium, or an admixture of the same, or their equivalents.

It will be evident that there are many methods of carrying my invention into practice, some of which are shown in the accompanying drawings; but I prefer turnings or cuttings of wire intimately mixed.

Numerous modifications both as regards the 90 configuration and disposition of the metal will suggest themselves to practical men, but those shown in the drawings are sufficient to allow

of the invention being carried into practice both as regards convenience to users and suitability of forms of scrap or metal easily obtained.

5 In all the views the same letters denote equivalent parts. *a*, surface of lining; *b*, body of lining; *c*, iron mixed with lining.

In Figure 1 the basic material is intimately mixed with turnings, short croppings of wire, or like small pieces of steel or iron. In Fig. 2 the base is mixed with and held together by metallic steel or iron wire twisted into serpentine forms placed lengthwise. In Fig. 3 involute coils of steel or iron wire are used. In Fig. 4 wire twisted helically is used. In Fig. 5 helices of wire are interlaced. In Fig. 6 helices of wire are crossed. In Fig. 7 matted or interlaced lengths of wire are used.

Fig. 8 is a cross-section of the hearth of a steel-furnace provided with my improved lining, the lining being the same as that shown in Fig. 1.

I claim—

1. A metallurgical furnace provided with a lime lining containing pieces of metallic iron or steel admixed therewith, substantially as and for the purposes described. 25

2. A basic lining for metallurgical furnaces, composed of lime admixed with pieces of metallic iron or steel, substantially as and for the purposes described. 30

W. F. BATHO.

Witnesses:

WM. THOS. MARSHALL,  
EDMUND S. SNEWIN.